

Patented June 22, 1926.

1,589,411

# UNITED STATES PATENT OFFICE.

LE ROY HIMES MINTON, OF METUCHEN, NEW JERSEY.

## NONSLIP TILE.

No Drawing.

Application filed August 24, 1925. Serial No. 52,224.

This invention relates to non-slip surfaces and particularly to ceramic floor-tile having rough relatively hard granular material embedded in the surface of the tile for the purpose of presenting a rough foot hold to pedestrians and preventing their slipping.

The granular material used in such tile must be hard enough to withstand the abrasion of passing feet without wearing down too rapidly. For this reason extremely hard materials have been used, such as previously fused alumina or silicon carbide, well-known as abrasives and having a hardness of 9 or more on Moh's scale. These materials serve the purpose, but in the form used, being artificial products and relatively expensive, serve perhaps too well. That is to say a hardness of 9 or more on Moh's scale is unnecessary and softer materials can serve equally well, provided they have the requisite toughness. A very hard but brittle material cannot stand up so well as one which is softer but tougher, and hence better able to withstand the shocks and strains of hard usage. Toughness is thus more important than hardness, provided of course, that the hardness is not too low. Materials having a hardness of less than 6 on Moh's scale are not best adapted for use as the non-slip elements of non-slip tile.

I have discovered that rutile serves excellently in the manufacture of non-slip tile and can well be substituted either in whole or in part for the harder and more expensive material heretofore used.

In making non-slip tile containing rutile as the non-slip element, I first reduce the

rutile to granular form of a fineness varying from 60 mesh to 12 mesh. This I add to a vitrifiable body made up of from 50% to 60% feldspar, 15% flint and the remainder ball clays, china clays, or kaolins, although the composition of the body may be varied and any good vitrifiable floor tile body employed. The quantity of rutile used may vary depending upon the degree of surface roughness required, but as practical limits I would set 20% and 80%. The rutile is preferably added to the body and thoroughly mixed with it just prior to the pressing operation. The tile are fired in the usual manner.

Rutile occurs naturally in relatively large quantities and is therefore inexpensive. It has a hardness on Moh's scale ranging from 6 to 6.5 and is sufficiently tough to resist the shocks to which floor tile are subjected. I have found that it forms a strong bond with the body of the tile and altogether performs the function of a non-slip element very satisfactorily.

I claim:

1. A non-slip surface having granular rutile embedded therein as a non-slip element.
2. A non-slip tile comprising a body of ceramic material having granular rutile embedded therein.
3. A non-slip tile comprising a vitrified floor tile body containing from 20% to 80% of granular rutile of a fineness varying from 60 to 12 mesh.

In testimony whereof I affix my signature.

LE ROY HIMES MINTON.